

Patented Feb. 17, 1948

2,436,007

500,000,000  
Aromatic primary amino developing agents  
containing an aryl group substituted with an  
alkoxy, carbethoxy acyl, acylanilido, or  
nitro group, and an R<sub>3</sub> group which is either a  
group of the same class as R<sub>2</sub> or is a hydrogen atom or a hydrocar-  
bon group.

Another group of U.S. patents from the same inventors  
J. D. Kendall and D. J. Fry, are U.S. Patents 2,436,007  
and 2,436,008. These patents are based on British Patents 615  
and 615A. The claims of these U.S. patents are as follows:

# UNITED STATES PATENT OFFICE

## DYE INTERMEDIATES FOR COLOUR PHOTOGRAPHY

John David Kendall and Douglas James Fry,  
Ilford, England, assignors to Ilford Limited,  
Ilford, England, a British company

No Drawing. Application May 3, 1945, Serial No.  
591,831. In Great Britain May 12, 1944

8 Claims. (Cl. 95—6)

This invention relates to colour photography  
and particularly to dyestuff intermediates for  
use in colour photographic processes.

Processes of colour photography are well known in which coloured images are produced by the development of reducible silver salt images by means of aromatic primary amino developing agents in the presence of compounds, generally known as "colour-formers" or "colour-couplers," which couple with the oxidation products of such developers, formed during development, to form quinone-imine or azomethine dyes. The colour-couplers may be present in the developing solution employed, or may be included in a photographic emulsion layer which contains the reducible silver salt image, or in an adjacent layer or a layer separated from the said emulsion layer only by a thin water-permeable layer. The developing agent may be, for example, p-phenylene diamine or its N,N-dialkyl derivatives, e. g., N,N-dimethyl or N,N-diethyl p-phenylene diamine, or homologues thereof, e. g., 5-diethylamino-2-aminotoluene.

Large numbers of colour-couplers have been described in the extensive literature dealing with this type of colour photographic process. The requirements for a satisfactory colour-coupler, however, are rather strict. Thus it must be capable of ready incorporation into the developing bath or photographic layer into which it is desired to include it, and where it is included in a photographic layer, neither it nor the dye derived from it must have any substantial tendency to diffuse from such layer, either into adjacent layers of the photographic element, or into processing baths. Moreover, it must be selected so that the colour of the dye obtained from it is suitable for the particular colour process with which it is intended to be used.

According to the present invention a process of colour photography comprises developing a reducible silver salt image by means of an aromatic primary amino developing agent in the presence of a compound of the general formula:

Another group of U.S. patents from the same inventors  
J. D. Kendall and D. J. Fry, are U.S. Patents 2,436,007  
and 2,436,008. These patents are based on British Patents 615  
and 615A. The claims of these U.S. patents are as follows:

where R<sub>1</sub> is an aryl group, R<sub>2</sub> is a —CN radical,

carboxy, alkoxy, carbethoxy acyl, acylanilido, or  
nitro group, and R<sub>3</sub> is either a group of the same  
class as R<sub>2</sub> or is a hydrogen atom or a hydrocar-  
bon group.

These compounds may be prepared by any con-  
venient method. A suitable method is by the  
condensation of an aryl acetaldehyde with a com-  
pound of the structure:

where R<sub>2</sub> and R<sub>3</sub> have the meanings assigned to  
them above. Thus, for example,  $\omega$ -cyan-allyl-  
benzene, C<sub>6</sub>H<sub>5</sub>CH<sub>2</sub>CH:CH.CN, may be prepared

by heating phenyl acetaldehyde with cyanacetic  
acid in pyridine solution. The reaction mixture  
is poured into water, the separated oil extracted  
with ether, the ether extracts dried, the ether  
distilled off and the residue redistilled (boiling  
range 180–200° C. 20 mm. pressure, solidifies  
on cooling). Similarly  $\omega$ -nitro-allyl-benzene,  
C<sub>6</sub>H<sub>5</sub>CH<sub>2</sub>CH:CH.NO<sub>2</sub> may be prepared using  
nitromethane instead of the cyanacetic acid

(boiling range 105–115° C. at 20 mm. pressure),  
and  $\gamma$ -phenyl ethylenemalonic diethyl ester,  
C<sub>6</sub>H<sub>5</sub>CH<sub>2</sub>CH:C(COOC<sub>2</sub>H<sub>5</sub>)<sub>2</sub>, may be similarly

prepared using diethyl malonate instead of the  
cyanacetic acid (boiling range 120–140° C., 20  
mm. pressure).

All these compounds yield good magenta  
images on colour-coupling development accord-  
ing to the invention.

Instead of phenyl acetaldehyde referred to  
above there may be employed, for example,  $\alpha$ -  
naphthyl acetaldehyde,  $\beta$ -naphthyl acetaldehyde,  
p-methoxyphenyl acetaldehyde, p-chlorophenyl

acetaldehyde, p-tolyl acetaldehyde, p-nitro-  
phenyl acetaldehyde or p-ethoxyphenyl acetal-  
dehyde. Other compounds for reaction there-  
with include cyan-, malonic- and aceto acetic  
esters and anilides, malodinitrile, cyanaceto-

hydrocarbons, coumarones, benzoyl-, furoyl- and  
picolinoylacetic esters and anilides, phenyl aceto-  
nitrile, diaroyl methanes, and quaternary salts  
of heterocyclic nitrogen compounds which con-  
tain a methyl group in  $\alpha$  or  $\gamma$  position to the  
quaternary nitrogen atom.

Particular compounds of use in the present invention are, for example:

Phenyl ethyldene cyanacetanilide



Phenyl ethyldene malodinitrile



p-Nitrophenyl ethyldene furoyl acetanilide



p-Chlorophenyl ethyldene dibenzoyl methane



p-Tolyl ethyldene cyanacetophthalene



The colour-couplers of this invention may be included in a developing solution containing an aromatic primary amino developing agent, or may be included in a silver halide emulsion layer, or in a water-permeable colloid layer coated next to a silver halide emulsion layer, or separated therefrom only by a thin water-permeable layer. Thus, for example, the colour-couplers of this invention may be used in any of the colour processes of U. S. Patents Nos. 2,350,380, 2,363,764 and 2,369,171, and British Patents Nos. 551,116, 551,117, 554,302 and 556,858.

The formation of coloured images by means of the colour-couplers of this invention may be applied to the development of a reducible silver salt image which is an original latent image formed in the emulsion layer by exposure to light or which is an image obtained by the conversion of a silver image to a reducible silver salt image by the usual bleaching technique.

Although this invention is primarily concerned with colour photographic processes in which the dye is formed by the coupling of the colour-couplers of the invention with the oxidation products of an aromatic primary amino developing agent formed in situ during the development of a reducible silver salt image, the colour-couplers of the invention may also be employed in other colour photographic processes e. g., processes in which the dye is formed by direct coupling between the colour-coupler and a nitroso aniline, e. g., p-nitroso dialkyl aniline, or between the colour-coupler and a diazo compound. As an example of this latter type of process a colour-coupler may be present in a layer containing a reducible silver salt image, such image developed with an aromatic primary amino developing agent forming an azomethine dye image in situ with the developed silver image, the residual colour-coupler coupled with a diazo compound applied in solution to the photographic element, and the original azomethine dye image bleached out, leaving only the azo dye image in the layer.

What we claim is:

1. A process of colour photography which comprises developing a reducible silver salt image in

a photographic element by means of an aromatic primary amino developing agent in the presence of a compound of the general formula:



where  $\text{R}_1$  is an aryl group,  $\text{R}_2$  is a group selected from the class consisting of —CN radicals, acyl, acylanilido, carboxy, alkoxy, carbethoxy, and nitro groups and  $\text{R}_3$  is a group selected from the class consisting of the hydrogen atom —CN radicals, acyl, acylanilido, carboxy, alkoxy, carbethoxy, nitro and hydrocarbon groups.

10 2. A process of colour photography which comprises developing a reducible silver salt in a photographic element by means of a solution of an aromatic primary amino developing agent containing a compound of the general formula:



where  $\text{R}_1$  is an aryl group,  $\text{R}_2$  is a group selected from the class consisting of —CN radicals, acyl, acylanilido, carboxy, alkoxy, carbethoxy, and nitro groups and  $\text{R}_3$  is a group selected from the class consisting of the hydrogen atom —CN radicals, acyl, acylanilido, carboxy, alkoxy, carbethoxy, nitro and hydrocarbon groups.

15 3. A photographic element for colour photography which comprises a support bearing at least one layer of a light-sensitive silver halide emulsion containing a compound of the general formula:



20 where  $\text{R}_1$  is an aryl group,  $\text{R}_2$  is a group selected from the class consisting of —CN radicals, acyl, acylanilido, carboxy, alkoxy, carbethoxy, and nitro groups and  $\text{R}_3$  is a group selected from the class consisting of the hydrogen atom —CN radicals, acyl, acylanilido, carboxy, alkoxy, carbethoxy, nitro and hydrocarbon groups.

25 4. A photographic element for colour photography which comprises a support bearing at least one layer of a light-sensitive silver halide emulsion and, adjacent thereto, a layer containing a compound of the general formula:



30 where  $\text{R}_1$  is an aryl group,  $\text{R}_2$  is a group selected from the class consisting of —CN radicals, acyl, acylanilido, carboxy, alkoxy, carbethoxy, and nitro groups and  $\text{R}_3$  is a group selected from the class consisting of the hydrogen atom —CN radicals, acyl, acylanilido, carboxy, alkoxy, carbethoxy, nitro and hydrocarbon groups.

35 5. A process of colour photography which comprises forming a reducible silver salt image in an emulsion layer of a photographic element which contains a compound of the general formula:



40 where  $\text{R}_1$  is an aryl group,  $\text{R}_2$  is a group selected from the class consisting of —CN radicals, acyl, acylanilido, carboxy, alkoxy, carbethoxy, and nitro groups and  $\text{R}_3$  is a group selected from the

